

## 1

3,307,900

## PROCESS FOR DYEING ACRYLONITRILE POLYMER FIBERS AND THEIR PRODUCTS

Ishihiko Nakanome and Tomoji Ohkubo, Saidaiji, Japan, assignors to Japan Exlan Company Limited, Osaka, Japan

No Drawing. Filed Dec. 2, 1963, Ser. No. 327,517  
Claims priority, application Japan, Dec. 6, 1962,

37/55,479

5 Claims. (Cl. 8—4)

This invention relates to a method of dyeing shaped articles comprising acrylonitrile polymers.

It is known to dye a shaped article comprising an acrylonitrile polymer by padding the article with a liquor containing a dyestuff and treating the wet article with steam to fix the dyestuff into the acrylonitrile polymer article. It is also known (U.S. Patent No. 2,654,652, patented October 6, 1953) to add a cyclic organic ester such as ethylene carbonate, gamma-butyrolactone, etc. in a padding liquor so as to improve the penetration of the dyestuff into the fiber. It is described in U.S. Patent No. 2,512,969 that meta-cresol is a good dye assistant in dyeing acrylonitrile polymer articles with dispersed or basic dyes in a boiling aqueous bath. However, meta-cresol is not effective when used in a pad-dyeing process as admitted in the above mentioned U.S. Patent No. 2,654,652 (column 2, lines 5—6).

The reasons why meta-cresol is not useful in a padding-steaming process while it is effective in a dip-dyeing process may be explained as follows: As is well known a more concentrated dye liquor is required in the case of padding-steaming method as compared with the case of dip-dyeing method, and consequently the concentration of dye assistant in the dye bath or padding liquor must also be higher. However, meta-cresol is comparatively low in water solubility so that when it is added in a large quantity to a padding liquor it will not disperse uniformly therein. When an acrylonitrile polymer article is immersed into such a padding liquor meta-cresol will deposit on the article unevenly so that the article with unevenly deposited meta-cresol is steam-treated resulting in dyeing defects such as uneven dyeing.

Accordingly, it is an object of this invention to provide a novel method for dyeing shaped articles comprising acrylonitrile polymers.

It is a more particular object of this invention to provide a satisfactory method for dyeing shaped articles of acrylonitrile polymers to uniformly and deeply dye the articles while using a cresol-containing padding liquor.

Other objects of this invention will be apparent from the following description.

Briefly, the objects of this invention are accomplished by padding a shaped article comprising an acrylonitrile polymer with an aqueous padding liquor containing a dyestuff and added with a cresol and an aliphatic polyhydric alcohol, and then treating the wet article with steam.

The present invention is applicable to shaped articles comprising acrylonitrile polymers. The polymers include not only polyacrylonitrile but also copolymers and graft copolymers of acrylonitrile with other monomers copolymerizable with acrylonitrile. The monomers copolymerizable with acrylonitrile are well known in the art and include, among others, vinyl acetate, vinyl chloride, vinyl pyridines such as 2-methyl-5-vinyl pyridine, acrylic acid

## 2

or its esters such as methyl acrylate, methacrylic acid or its esters such as methyl methacrylate, methacryl sulfonic acid or its salts, and other similar polymerizable hydrocarbons and their derivatives. In any case, it is preferable that acrylonitrile polymers contain at least 40% by weight of acrylonitrile component.

Any shaped articles may be used. Thus, for example, they may be films, fibers, fiber tow, yarns, woven fabrics, knit fabrics, and made-up articles of clothing.

10 The dye bath or padding liquor may contain any dyestuff which has conventionally been used in dyeing acrylic fibers. Among dyestuffs useful in this invention are cationic dyestuffs, acidic dyestuffs and metal-containing dyestuffs. If desired a mixture of suitable dyestuffs may also be used.

The concentration of dyestuff in the aqueous padding liquor is not critical, although it is preferable to be higher than in the usual dip-dyeing bath. Generally, a concentration of from 10 to 50 g. per liter is satisfactory, although any higher concentration may be used where such a higher concentration is required to obtain desired shade.

The important feature of the invention is that the padding liquor also contains a cresol and an aliphatic polyhydric alcohol.

25 Any of the cresols including o-cresol, m-cresol and p-cresol may be used. If desired a mixture of any two or more of these cresols may also be used.

The aqueous dye bath or padding liquor should contain at least 30 g. of cresol per liter of the liquor. Generally, it is preferable that the cresol concentration is 50—100 g. per liter of the padding liquor.

30 Aliphatic polyhydric alcohols which are used in this invention contain not more than 6 carbon atoms. Among aliphatic polyhydric alcohols useful in this invention are dihydric alcohols such as ethylene glycol, diethylene glycol, propylene glycol, pentamethylene glycol, hexamethylene glycol, etc., trivalent alcohols such as glycerine, butane triol, pentane triol, etc., tetra-valent alcohols such as erythrite, pentaerythrite, etc., among which, however, ethylene glycol, diethylene glycol and propylene glycol are preferable. In order to uniformly disperse cresol in the padding liquor the amount of the polyhydric alcohol should be at least two times (by weight) that of cresol. Generally, the use of a polyhydric alcohol in an amount from 2 to 3 times by weight based on cresol is satisfactory, but no adverse effect is seen when a larger amount is added. Of course, a mixture of any two or more of the above mentioned aliphatic polyhydric alcohols may also be used.

35 40 45 50 55 60 65 The temperature of the padding liquor is not critical. Thus it may be room or ordinary temperature. However, when the dye concentration is high it is preferable to heat (e.g. 30—40° C. and up to about 60° C.) the padding liquor to prevent precipitation of the dyestuff.

In carrying out the method of this invention, a shaped article comprising an acrylonitrile polymer is padded with the above mentioned padding liquor. This may be conducted in a known manner for example by immersing the article in the padding bath.

The amount of dye or padding liquor to be picked up by the article may vary depending upon the desired depth of shade, concentration of the dye in the liquor and generally the pick-up may be within a range from 70 to 120%, but usually a pick-up of about 100% is satisfactory.

Then the article thus padded with the aqueous dye liquor is subjected to a steam treatment. The wet steam treat-

ment is carried out in steam of a temperature of from 100° C. to 150° C. The time of this steam treatment may vary depending upon the particular steam temperature and should be sufficient to obtain the desired result. Generally the steam treatment of at least 30 seconds is necessary. For example, when the steam treatment is carried out at a temperature of from 100° C. to 105° C. a satisfactory result would be obtained in about 0.5-2 minutes.

After the steam treatment, the dyed article is finished in a usual manner. Thus the dyed article is washed with water to remove any dye, cresol and alcohol which remain on the article surface. In case of deep dyeing, it is preferable to treat the dyed article with an aqueous liquor containing soap or non-ionic surfactant in an amount of 0.5 g./l. at about 60° C. for about 15 minutes and then to wash with water. The washed article is then dried, e.g. at about 80-100° C. for about 5-10 minutes.

According to this invention, shaped articles comprising acrylonitrile polymers can readily be dyed deeply and uniformly without using any special apparatus.

The invention will be better understood when referred to the following examples which are given for illustrative purposes only and are not limitative in any way. In these examples, all parts and percentages are by weight. The colorimetric test was carried out by dissolving 0.02 g. of the dyed sample in 20 g. of gamma-butyrolactone and measuring the light absorbency of the solution with a photoelectric colorimeter (FPW-III type colorimeter of Hitachi Seisakusko) with the filter indicated.

#### Example 1

In 1000 parts of water was dissolved 25 parts of C. I. Basic Yellow 23 to prepare an aqueous dye solution. Then a mixture of 100 parts of a mixture of o-, m- p-cresols and 300 parts of ethylene glycol was added to the above dye solution.

A tow of fibers prepared from a copolymer of 90% acrylonitrile and 10% methyl acrylate was immersed in the above mentioned padding liquor and squeezed to a pick-up of 100%. The wet padded tow was treated for 30 seconds to 10 minutes with steam of 100° C. and then washed with water and dried.

The same procedure was repeated except that the mixture of cresols and ethylene glycol was not added to the padding liquor.

The dyed fibers thus obtained were subjected to a colorimetric examination and the following results were obtained.

| Steaming time (minutes) | Control, no dye assistant added | Cresol and ethylene glycol added |
|-------------------------|---------------------------------|----------------------------------|
| 0.5                     | 0.096                           | 0.305                            |
| 1.0                     | 0.252                           | 0.510                            |
| 2.5                     | 0.362                           | 0.608                            |
| 5.0                     | 0.478                           | 0.650                            |
| 7.5                     | 0.500                           | 0.670                            |
| 10.0                    | 0.581                           | 0.685                            |

Remarks: A filter of 430 m $\mu$  was employed.

It will be apparent from the above table that when cresol and ethylene glycol are added to the padding liquor the dye absorbency of the fiber is remarkably improved and the time required for steaming is substantially reduced as compared with the case where no such cresol and ethylene glycol was added.

When only cresol was added and ethylene glycol was not added in the above example, the fibers were dyed too unevenly to be of commercial value.

#### Example 2

In 1000 parts of water was dissolved 25 parts of C. I. Basic Red 14 to prepare an aqueous dye solution. Then

5

a mixture of 100 parts of m-cresol and 300 parts of ethylene glycol was added to the above dye solution.

A tow of fibers prepared from a copolymer of 90% acrylonitrile and 10% methyl acrylate was immersed in the above prepared padding liquor and then treated in the same manner as in Example 1.

The same procedure was repeated but without adding the mixture of m-cresol and ethylene glycol to the padding liquor.

The dyed fibers thus obtained were subjected to a colorimetric examination and the following results were obtained.

| Steaming time (minutes) | Control, no dye assistant added | Cresol and ethylene glycol added |
|-------------------------|---------------------------------|----------------------------------|
| 0.5                     | 0.072                           | 0.407                            |
| 1.0                     | 0.165                           | 0.480                            |
| 2.5                     | 0.302                           | 0.688                            |
| 5.0                     | 0.462                           | 0.780                            |
| 7.5                     | 0.490                           | 0.790                            |
| 10.0                    | 0.505                           | 0.800                            |

Remarks: A filter of 500 m $\mu$  was employed.

#### Example 3

In 1000 parts of water was dissolved 25 parts of C. I. Basic Blue 54 and a mixture of cresol (o-, p-, m-cresols mixture) 100 parts and diethylene glycol 300 parts was added thereto to prepare a padding liquor.

A tow of fibers prepared from a copolymer of 90% acrylonitrile, 9.5% methyl acrylate and 0.5% sodium methallyl sulfonate was immersed in the above padding liquor and squeezed to a pick-up of 100%. The wet padded fiber tow was treated for 2 minutes with steam at 105° C., and then washed with water and dried. The fiber was evenly dyed in a deep blue shade.

25

30

35

40

45

50

#### Example 4

A fabric prepared from yarn of a copolymer of 90% acrylonitrile, 5% vinyl acetate and 5% 2-methyl-5-vinyl pyridine was a padded with an aqueous padding liquor containing 100 g. of C. I. Acid Blue 23 (C. I. No. 61,215), 20 g. of sulfuric acid (98%), 100 g. of cresol (o-, m- and p-cresols mixture) and 300 g. of propylene glycol per liter of the bath. The fabric with a pick-up of 100% was treated for 2 minutes with steam at 105° C., and then washed with water and dried. The fabric was evenly dyed in a deep blue shade.

#### Example 5

A fabric prepared from yarn of a copolymer of 90% acrylonitrile and 10% methyl methacrylate was padded with an aqueous padding liquor containing 5 g. of C. I. Basic Orange (C. I. No. 48,035), 5 g. of C. I. Basic Blue 45, 10 g. of acetic acid, 50 g. of (o-, m- and p-cresols mixture) cresol and 150 g. of ethylene glycol per liter of the bath. The fabric was squeezed to a pick-up of 100% and treated for 3 minutes with steam at 105° C. Then the steam treated fabric was soaped with nonionic surface active agent, washed with water and dried. The fabric was evenly dyed in an exceptionally vivid khaki shade.

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

44

of the cresol is at least 30 grams, per liter of the padding liquor.

3. A method as claimed in claim 1 in which the amount of the cresol is from 50 to 100 grams per liter of the padding liquor.

4. A method as claimed in claim 1, in which the steaming is carried out at a temperature of from 100° C. to 150° C.

5. A method as claimed in claim 1 in which the aliphatic polyhydric alcohol is selected from the group consisting of ethylene glycol, diethylene glycol and propylene glycol.

**References Cited by the Examiner**

**UNITED STATES PATENTS**

|           |         |           |       |      |
|-----------|---------|-----------|-------|------|
| 2,512,969 | 6/1950  | Richards  | ----- | 8—4  |
| 2,558,735 | 7/1951  | Cresswell | ----- | 8—55 |
| 2,717,823 | 9/1955  | Lowe      | ----- | 8—55 |
| 2,812,230 | 11/1957 | Evans     | ----- | 8—55 |

NORMAN G. TORCHIN, *Primary Examiner.*

10 J. TRAVIS BROWN, *Examiner.*

T. J. HERBERT, *Assistant Examiner.*